

Jan. 13, 1953

G. A. RICHTER, JR., ET AL  
PROCESS FOR PRODUCING REGENERATED  
CELLULOSE ARTICLES FROM VISCOSE  
Filed Oct. 2, 1950

2,625,461



FIG. 1



FIG. 2



FIG. 3



FIG. 4

INVENTORS.  
GEORGE ALVIN RICHTER, JR.  
RICHARD H. BRAUNLICH

BY *Thomas B. Mallon*  
ATTORNEY.

## UNITED STATES PATENT OFFICE

2,625,461

PROCESS FOR PRODUCING REGENERATED  
CELLULOSE ARTICLES FROM VISCOSEGeorge A. Richter, Jr., Springfield, and Richard  
H. Braunlich, West Chester, Pa., assignors to  
American Viscose Corporation, Wilmington,  
Del., a corporation of Delaware

Application October 2, 1950, Serial No. 187,858

20 Claims. (Cl. 18—54)

1

This invention relates to the manufacture of artificial filaments and fibers from viscose. More particularly, it relates to a novel two-stage spinning process for the production of regenerated cellulose fibers. By the term "two-stage spinning" is meant that type of process in which the viscose is first coagulated with little or no regeneration and this is followed by a subsequent stage of regeneration.

This application is a continuation in part of our application, Serial No. 128,382, filed November 19, 1949, entitled "Process for Producing Regenerated Cellulose Articles From Viscose," now abandoned.

It has been recognized in the patent and technical literature that artificial filaments can be formed by spinning viscose into a bath containing phosphate ions. For example, if viscose is spun into a coagulating bath containing sodium phosphates and sodium sulfate, cellulose xanthate threads are obtained which can then be stretched and treated with a medium for hydrolyzing cellulose xanthate to cellulose. This constitutes what is known as a "two-stage process." However, while such two-stage procedures have been known, they have remained more or less laboratory curiosities due to their high cost and impracticality. In such previously known systems, all of the sodium hydroxide entering the system with the viscose has generally been neutralized by phosphate salts or phosphoric acid, which are prohibitively expensive as compared to the sulfuric acid which is used as the neutralization agent in conventional viscose spinning in which coagulation and regeneration are performed in a single step in a single bath. A separate recovery system for phosphoric acid or phosphate salts would be necessary, but the added expense and trouble thereby entailed prevents the products obtained by such systems from becoming competitive with those from the single-stage sulfuric acid systems from the standpoint of cost.

One object of this invention is to provide a simple, readily controllable, economically feasible, continuous two-stage phosphate system for producing fibers from viscose.

By the present invention, the disadvantages which formerly attended the execution of the two-stage phosphate process are eliminated because the coagulating bath containing the phosphoric acid and/or sodium phosphates, and the regenerating bath, are integrated into a simple, practical, economical and novel two-stage system in which a phosphate bath serves to dehydrate the viscose filament-forming streams and as a vehicle to carry hydrogen ions to the viscose filament-forming streams for neutralizing the sodium hy-

2

droxide thereof, thereby coagulating them, and the phosphate bath is maintained at, or reconverted to, its initial coagulating effectiveness by the addition of sulfuric acid to the two-stage system. In effect, it is the sulfuric acid that is consumed for the neutralization of virtually all of the sodium hydroxide in the viscose.

The invention will be described with reference to the accompanying drawing, in which

Fig. 1 illustrates schematically the flow of various streams through the system;

Fig. 2 is a diagrammatic elevation of apparatus suitable for use in practicing one embodiment of the invention;

Fig. 3 is a diagrammatic elevation of apparatus suitable for use in practicing another embodiment of the invention; and

Fig. 4 is a diagrammatic elevation of apparatus suitable for use in practicing a further embodiment of the invention.

In Fig. 1 of the drawing, A represents the storage and make-up tank for the coagulating bath which comprises an aqueous solution of sodium sulfate and an acid sodium phosphate and which may also contain phosphoric acid, and B represents the vessel into which the viscose is spun. The coagulating bath is circulated between tank A and vessel B in streams 9 and 10. C represents the storage and make-up tank for the regenerating bath, the composition of which is discussed below, and D represents the vessel containing regenerating bath through which the coagulated cellulose xanthate thread is passed to initiate rapid regeneration of the cellulose. The regenerating bath is circulated between tank C and vessel D in streams 11 and 12.

In accordance with the broader aspects of the invention, viscose (stream 2 in Fig. 1) is extruded through a spinneret 20 into the coagulating bath in vessel B. The bundle of cellulose xanthate filaments thus formed is drawn from the coagulating bath, stripped of excess coagulating bath, and passed through a regenerating bath contained in vessel D. After the thread is withdrawn from vessel D, it preferably passes through a stripping device and out of the system (stream 4) and may be then desulfided, bleached, washed, treated with a finish, dried, and collected in continuous manner; if desired, it may be cut into staple fiber before or after these liquid-treating and drying steps.

If desired, no stretch need be performed on the filaments except that which would occur between the jet and first draw-off device, but for most purposes, a stretch of at least 40%, and preferably 100% to 200% or more, is applied after the thread leaves the coagulating bath. The fila-

ments or threads may be stretched between the coagulating and regenerating bath, as they enter the regenerating bath or as they are passed through the regenerating bath.

In the preferred embodiment, the coagulated cellulose xanthate filaments are stretched between the coagulating and regenerating baths and relaxed during their passage through the regenerating bath so that regeneration of the cellulose is effected while the filaments are relaxed. Such filaments are less brittle and more readily workable on conventional textile working equipment than the filaments which are stretched simultaneously with regeneration.

Apparatus for carrying out the preferred embodiment is shown in Fig. 2. Referring to Fig. 2, the coagulated cellulose xanthate filaments are shown proceeding from the coagulating bath contained in vessel B over the guide 22, to the godet 23 and thence to godet 30. As they proceed from godet 23 to godet 30, the filaments are passed between stripping guides 24 and 25 arranged in staggered relation to strip excess coagulating liquid therefrom. Between godets 23 and 30, the filaments are stretched to the desired extent. The stretched filaments proceed from godet 30 and through the regenerating bath contained in vessel D, and are withdrawn from the regenerating bath over the guide 27, and passed between the stripping guides 28, 29 arranged in staggered relation to strip excess regenerating liquid from the filaments, and thence to the godet 31. From godet 31 the thread passes out of the system (stream 4) and may then be desulfided, bleached, washed, treated with a finish, dried, and collected in continuous manner; if desired, it may be cut into staple fiber before or after these liquid-treating and drying steps.

In order to insure relaxation of the filaments in the yarn or tow during regeneration of the cellulose in vessel D, godet 31 is driven at a lower peripheral speed than godet 30. Generally, the peripheral speed of godet 31 (linear speed of yarn) is from 1 to 3% slower than that of godet 30, the thread being relaxed from 1 to 3% as it passes through the regenerating bath. The thread can be relaxed more than 3% during passage thereof through the regenerating bath contained in vessel D, if desired.

In the embodiment shown in Fig. 3 of the drawing, the thread is stretched simultaneously with regeneration of the cellulose. As shown, the thread is withdrawn from the coagulating bath in vessel B over the guide 22 to godet 23 (godet 30 is omitted in this modification of the invention) and passes between the stripping guides 24 and 25 arranged in staggered relation. From guides 24 and 25, the filaments pass into and through the regenerating bath in vessel D, and are withdrawn from the regenerating bath over guide 27, and passed between the stripping guides 28 and 29, to the godet 31.

In order to stretch the thread to the desired extent as it is passed through the regenerating bath, godet 31 is driven at a higher peripheral speed than godet 23. From godet 31 the thread passes out of the system (stream 4) to the after-treating stages as referred to in connection with Fig. 1.

In the several embodiments hereinabove the jet-velocity: draw-off ratio may have any of the conventional values, such as 1:3 to 1:0.3. However, for special purposes ratios outside this range may be used. For example, the process of this invention is adaptable to the production of

crimped regenerated cellulose filaments by methods involving the spinning of viscose with an exceptionally high jet-velocity: draw-off ratio. Such crimped filaments can be obtained by extruding the viscose into a phosphate coagulating bath as disclosed herein at a high velocity of extrusion, withdrawing the coagulated cellulose xanthate filaments at a low velocity of draw-off, stretching the coagulated xanthate filaments at least 25% over their straight length (i. e. to 125% of their original length), and regenerating and drying the stretched filaments in a relaxed condition. The velocity of extrusion of the viscose into the phosphate coagulating bath is preferably at least four times the velocity of draw-off.

Apparatus suitable for use in practicing the last-mentioned embodiment of the invention is shown in Fig. 4. Referring to Fig. 4, the viscose filament-forming composition is forced through the spinneret 20 into the phosphate coagulating bath contained in vessel B under sufficient pressure that the velocity of extrusion of the filaments is at least four times the velocity of draw-off by the godet 23. The filamentous solution buckles and bends as it is forced into the coagulating bath in vessel B, thus forming highly crimped filaments of cellulose xanthate. The filaments are withdrawn from vessel B over the guide 22 by the godet 23 and passed to godet 30 between the stripping guides 24 and 25. Godet 30 is driven at a higher peripheral speed than godet 23, whereby the filaments are stretched at least 25% over their straight length. From godet 30, the filaments drop into and through the regenerating bath contained in vessel D from which they are withdrawn over guide 27 and passed to godet 31 between the staggered stripping guides 28 and 29. Godet 31 is driven at a lower peripheral speed than godet 30, so that the filaments dropped into vessel D tend to pile up on one side of the partition 32 which extends to within a short distance of the bottom wall of the vessel. The filaments pass under the partition, and under the guide 33 submerged in the regenerating bath, the regeneration thus being effected while the filaments, yarn, or tow are in a relaxed condition. The thread leaves the system (stream 4) and proceeds to the after-treating stages. It may be after-treated, i. e., purified and washed in relaxed condition, or under tension, but in any case it is dried in the relaxed condition to permit the free formation of crimp.

This invention is concerned more particularly with the manner in which the non-cellulosic portions of streams 2 to 19 (Fig. 1) are manipulated, and especially with the reactions resulting in the consumption of sulfuric acid exclusively for the neutralization of the sodium hydroxide introduced into the system with the viscose.

In the present process, the coagulating bath may have a pH of 1.5 to 10. When operated in the pH range of 3.7 to 9 in the coagulating bath, the sodium hydroxide reacts with mono-basic sodium phosphate obtained by the reaction of sulfuric acid with dibasic sodium phosphate, the mono- and di-basic sodium phosphates being continuously reversibly converted in the system from one to the other.

Thus, when the viscose is introduced into the coagulating bath containing mono-basic sodium phosphate, the sodium hydroxide reacts with the mono-basic sodium phosphate according to the following reaction:



When operated at a pH of less than 3.7, for example, at a pH between 1.5 and 3.7, the reaction also involves the conversion, by the sodium hydroxide in the viscose, of some phosphoric acid to mono-basic sodium phosphate. When operated at a pH for the coagulating bath between 9 and 10, the reaction also involves the conversion of dibasic sodium phosphate to tri-basic sodium phosphate.

The cellulose xanthate thread passing from the coagulating bath to the regenerating bath contained in vessel D carries with it from the coagulating bath a substantial amount of solution, usually about 6 to 10 pounds of solution per pound of cellulose, which solution comprises mono- and/or di-basic sodium phosphate, sodium sulfate, by-product sulfur compounds, and water, with or without free phosphoric acid depending on the pH of the coagulating bath. The solution is carried by the thread to vessel D and introduced into the regenerating bath which, at the start of operations comprises an aqueous solution of sulfuric acid, phosphoric acid, and sodium sulfate. Sufficient free sulfuric acid is maintained therein to convert the phosphate salts in the thread at least partially to phosphoric acid, whereby sufficient acid is carried by the thread bundle to assure the complete regeneration of the sodium cellulose xanthate to cellulose. The reconversion of the phosphate salts takes place in accordance with the following reactions:



Enough acid is added here to convert all of the sodium phosphates in the body of the regenerating bath to phosphoric acid. Preferably the concentration of sulfuric acid in the regenerating bath is maintained slightly below the concentration thereof required to convert all of the phosphate salts in the yarn bundle to phosphoric acid, so that mechanical loss of sulfuric acid by removal thereof in stream 4 is avoided.

The concentrations of phosphoric acid and sodium sulfate in the regenerating bath are allowed to reach equilibrium values determined by the amount and composition of the solutions constituting streams 3 and 4. Under the preferred ranges of spinning conditions, the equilibrium concentrations of phosphoric acid and sodium sulfate in the regenerating bath are in the ranges 5 to 10% and 10 to 20% respectively.

Because of the highly swollen condition of the xanthate yarn leaving the coagulating bath, the amount of liquid carried from vessel B by the cellulose xanthate threads (stream 3) and introduced into vessel D is greater than the amount of liquid carried from the system by the less highly swollen yarn undergoing regeneration (stream 4), and therefore, the regenerating bath builds up in vessel C as spinning proceeds. All or a portion of the excess regenerating bath thus accumulated is passed, continuously or intermittently, from vessel C to the coagulating bath, for example to that in storage tank A (stream 7). The phosphoric and sulfuric acids present in this circulated liquid function to reconvert some of the tribasic, dibasic, or mono-basic sodium phosphate produced by reaction (1) to dibasic sodium phosphate, monobasic sodium phosphate, or free phosphoric acid respectively. The following reactions are illustrative when operating in the pH range of 3.7 to 9:



Phosphoric acid is introduced into tank A (stream 9a) only in the amount necessary to replace the phosphate ions lost mechanically by removal of phosphoric acid in stream 4. This is supplemented with sulfuric acid (stream 8) as required to complete reconversion in tank A of the respective sodium phosphate to the more acid form of sodium phosphate or to phosphoric acid itself to maintain or restore the initial pH value of the coagulating bath before returning it to vessel B. In place of phosphoric acid in stream 9a, other forms of phosphate such as one or more of the sodium phosphates, may be present in that stream.

The excess sodium sulfate (corresponding to the amount formed by the neutralization of sodium hydroxide in the viscose) which accumulates in the coagulating bath as a result of these reactions is removed continuously or intermittently by crystallization of Glaubers salt in a crystallizer K (stream 5). In the preferred modification, the pH of the solution withdrawn from tank A (by stream 13) for crystallization of the decahydrate is adjusted to 5.5 or below, for example by the addition of sulfuric acid to it (stream 14). Under these conditions, crystallization of the sodium sulfate in stream 5 takes place preferentially, with substantially no crystallization of phosphate radicals. The liquid remaining from the crystallization is returned to tank A (stream 15).

Excess water is evaporated from the coagulating bath by intermittently withdrawing a portion thereof (stream 16) to an evaporator E, and the bath, freed of excess water, is returned to tank A (stream 17). If desired, stream 15 may be diverted to an evaporator, such as E, to remove excess water before it is returned to tank A. The excess water removed corresponds to the sum of the water introduced by streams 2, 6, 8, 9 and neutralization of sodium hydroxide in the viscose minus the sum of the water removed in streams 4 and 5.

In order to operate economically in accordance with this invention, the amount of solution carried by the xanthate fibers into the regenerating bath in vessel D must be controlled because, if it is excessive, the amount of sulfuric acid which must be added to vessel C (stream 6) to convert at least a portion of the phosphate salts in the yarn bundle to phosphoric acid is so high that the pH balance in the coagulating bath is upset when the total overflow from vessel C is circulated to tank A (stream 7). To avoid such an upset, a portion only of stream 7 may be introduced directly into tank A. However, in the preferred embodiment, if the amount of solution in stream 3 is excessive under the selected operating conditions, some of the solution is stripped from the cellulose xanthate thread proceeding from B to D and allowed to flow back into the coagulating bath, either in vessel B or tank A, as shown (stream 18). The minimum amount of solution which it may be necessary to strip off the xanthate threads depends on the composition of streams 3 and 4. Efficient stripping of the xanthate threads also results in lower equilibrium values for the phosphoric acid and sodium sulfate concentrations in the regenerating bath, and in rapid absorption of the regenerating bath by the yarn bundle whereby regeneration of the cellulose xanthate to cellulose is accelerated. In general, if the weight ratio of solution to cellulose in stream 3 is maintained at 8:1 or less, all of stream 7 may be introduced directly into tank A.

The amount of solution carried by the thread in stream 3 into the regenerating bath and the amount of sulfuric acid in stream 6 may be correlated so that when all of the excess regenerating bath is cycled back to tank A by stream 1, no additional sulfuric acid need be added to the coagulating bath and stream 8 may be omitted. The preferred system involves stripping of stream 3 to minimize loss of phosphate in stream 4.

As previously noted, the coagulating bath comprises an aqueous solution of sodium sulfate and sodium phosphates, and may also contain phosphoric acid. Some latitude in the actual composition of the bath is permissible, so long as the acid in the overflow from the regenerating bath storage tank C to tank A (stream 7) does not overcompensate for the sodium hydroxide entering the system with the viscose. The coagulating bath has a pH of 1.5 to 10 and contains phosphate radicals in a selected proportion between 5 and 20% by weight, and sodium sulfate in a selected proportion between 5 and 20%, by weight, the conditions selected being maintained throughout the spinning. The temperature of the coagulating bath may be room temperature or higher and is preferably between 45 and 55° C. The immersion length for the fibers in the coagulating bath is not critical, and may be, for instance, between 12 and 20 inches.

When the concentrations of sodium sulfate and phosphate radicals in the coagulating bath are kept within the ranges just specified and the ratio of solution to cellulose in stream 3 is not greater than 8:1, the sulfuric acid content of the regenerating bath may be maintained at about 1 to 15% by weight and preferably 3 to 6%, and the equilibrium values for phosphoric acid and sodium sulfate in the regenerating bath are 5 to 10%, and 10 to 20%, respectively. The regenerating bath may have room temperature or higher and preferably has a temperature of from 45 to 55° C.

The viscose may be a normal viscose that is, it may have a salt point of 3 to 6 (sodium chloride salt test value), a cellulose content of from 6 to 9%, and a sodium hydroxide content of from 6 to 9%. The viscosity may be normal, also, that is between 30 and 60 seconds as measured by the ball fall test. However, it is preferred to use a viscose of higher viscosity, for example, one having a ball fall viscosity of 65 to 120 seconds, and, consequently, a higher degree of polymerization. Such viscoses are obtained by reducing the storage time of the soda cellulose crumbs, as is well known. The cellulose used in making the viscose may be of cotton or wood origin or any mixture of the two.

The fibers leaving the regenerating bath are sent directly to the usual finishing stages through which regenerated cellulose fibers are passed in the normal course of their production.

The fibers exhibit high tensile strengths (wet and dry) combined with low extensibilities (wet and dry) and low swellings (cross-sectional and linear) upon exposure to water or water vapor. Average fiber properties are tabulated below:

|                                |                         |
|--------------------------------|-------------------------|
| Tenacity (dry) .....           | 3.3 to 4.5 grams/denier |
| Tenacity (wet) .....           | 2.0 to 3.0 grams/denier |
| Extensibility (dry) .....      | 7.0 to 8.5%             |
| Extensibility (wet) .....      | 7.0 to 8.0%             |
| Cross-sectional swelling ..... | 40%                     |
| Linear swelling .....          | 0.25%                   |
| Young's modulus (wet) .....    | 20                      |

In the following examples, specific embodiments of the novel two-stage process of the invention are described with reference to the figures of the drawing designated.

5

*Example 1*

A 100% cotton viscose having a sodium chloride salt test value of  $6 \pm 0.5$ , a ball fall viscosity of 75 seconds at 21° C. (soda cellulose storage time at 21° C.: 36 hours), and containing 7.8% cellulose, 38%  $\text{CS}_2$  (based on the cellulose), and 6.6% sodium hydroxide was pumped through a spinneret 20 containing 980 orifices, each 0.0025 inch in diameter, into an aqueous coagulating bath contained in vessel B in the system of Figures 1 and 3, and comprising a solution containing, by weight 11.9  $\pm 0.5$  % phosphate radicals (as mono- and di-sodium phosphates) and 10.0  $\pm 1.0$  % sodium sulfate at a pH of  $5.0 \pm 0.2$  and a temperature of 50° C. After an immersion of 12 inches, the cellulose xanthate filaments were withdrawn from the bath over guide 22, lapped around godet 23, passed through vessel D containing the regenerating bath (immersion distance: 30 inches), withdrawn over the guide 27 between the stripping guides 28 and 29, arranged in staggered relation beyond the regenerating bath to strip the fibers of excess solution, to the godet 31. The solution stripped from the yarn tow between guides 24 and 25, and guides 28 and 29 was returned to the coagulating and regenerating baths respectively in streams 18 and 19, as shown in Fig. 1. The fibers advancing from the coagulating bath contain approximately ten pounds of coagulating liquid per pound of cellulose. After stripping by the staggered guides 24 and 25, the fibers contained approximately seven pounds of coagulating liquid per pound of cellulose. The fibers were stretched 210% between godets 23 and 31. The spinning speed at godet 31 was 60 meters per minute.

Initially the regenerating bath, which was maintained at 50° C., consisted of water containing 5% sulfuric acid, 7% phosphoric acid and 18% sodium sulfate. These are the equilibrium values for phosphoric acid and sodium sulfate as calculated from analysis data on the cellulose xanthate thread (stream 3 of Figure 1) after stripping thereof between guides 24, 25, and on the cellulose thread (stream 4 of Figure 1) after stripping thereof by the guides 28 and 29. The regenerating bath volume was kept constant by replacing water lost by evaporation and returning the overflow (stream 7 of Figure 1) to the coagulating bath at the rate of 2.4 lbs. per pound of bone dry yarn produced. This overflow from the regenerating bath to the coagulating bath assists in maintaining the coagulating bath composition and pH constant. However, in addition to the reagents cycled from the regenerating bath to the coagulating bath, the coagulating bath was intermittently fortified by the addition of 4.3 lbs of 94% sulfuric acid (stream 8 of Figure 1) at regular six-hour intervals (0.33 lb. of sulfuric acid per pound of bone dry yarn produced) and 5.9 lbs. of 85% phosphoric acid (stream 9a of Figure 1) at regular six-hour intervals (0.42 lb. of phosphoric acid per pound of bone dry yarn produced). Nine pounds of 94% sulfuric acid were added to the regenerating bath in tank C (stream 6 of Figure 1) at regular 12 hour intervals (0.73 lb. of sulfuric acid per pound of bone dry yarn produced) to maintain the concentration of free sulfuric acid in the regenerating bath at 5%.

75 The concentrations of sodium sulfate and

phosphoric acid in the regenerating bath, calculated as equilibrium values at the start, remained substantially constant. The coagulating bath was drawn off intermittently to a vacuum crystallizer K (Figure 1) for crystallization of the excess sodium sulfate accumulated in the system. The excess water built up in the system was evaporated in evaporator E (Figure 1).

The fibers, after the usual after-treatments including desulfiding, bleaching, washing and drying, were highly crystalline as shown by X-ray and hydrolysis rate studies. The dry and wet tenacities of the fibers were 4.3 gms./denier and 2.6 gms./denier, respectively. The dry and wet extensibilities were 8.7% and 9.5%, respectively. The cross-sectional swelling is in the range of 40 to 45%; linear swelling about 0.25%.

*Example II*

Example I is repeated, using the system of Figures 1 and 2 of the drawing. The viscose was pumped into the coagulating bath in vessel B, withdrawn over the guide 22, lapped around godet 23, passed to godet 30 between the stripping guides 24 and 25 and stretched 102% between the godets. From godet 30, the yarn comprising the cellulose xanthate filaments was passed through vessel D containing the regenerating bath (immersion distance: 30 inches), withdrawn over the guide 27, and passed between the stripping guides 28 and 29 to godet 31. Godet 31 was driven at a peripheral speed such that during passage of the filaments through the regenerating liquid in vessel D they were relaxed 3%. A yarn produced as described in this example had the following properties:

|                          |      |
|--------------------------|------|
| Total denier             | 1572 |
| Denier/filament          | 1.61 |
| Tenacity in gms./denier: |      |
| Dry                      | 3.4  |
| Wet                      | 2.0  |
| Extensibility:           |      |
| Dry                      | 8.5  |
| Wet                      | 8.0  |

The yarn or filaments were found to be less brittle than the filaments or yarn of Example I.

*Example III*

Example II was repeated using the system of Figs. 1 and 4. The viscose was extruded into the coagulating bath in vessel B at an extrusion velocity four times greater than the rate at which the filaments were withdrawn from the bath by godet 23. The filaments were stretched 125% between godets 23 and 30 and allowed to fall into the regenerating bath contained in vessel D. The filaments passed under the partition 32 and the guide roll 33, and were withdrawn from the regenerating bath over the guide 27, and passed between the stripping guides 28 and 29 to godet 31. Godet 31 was driven at a lower speed than godet 30, to permit free relaxation of the filaments during their passage through the regenerating bath. The filaments were then removed from the system (stream 4 of Fig. 1) and subjected to the usual after-treating liquids including desulfiding, bleaching, washing and drying. These liquid after-treatments and the drying were performed while the yarn comprising the filaments was in skein form and free to relax. Crimped filaments or yarn are obtained by this process.

Some modification of the coagulating bath is permissible. Thus, a small proportion of a sur-

face-active agent which is inert to the constituents of the bath may be added for preventing spinneret incrustation.

If desired, in carrying out this process, the viscose may be extruded into the coagulating bath in vessel B in a pulsating manner, i. e., the viscose may be delivered to the spinneret at a varying rate to produce filaments having irregular denier along their length, sections along the filament of heavier denier, which may be called "nubs" or "slubs" alternating with sections of lighter denier. Such irregular filaments may have particular advantages. Examples of apparatus suitable for varying the rate of delivery of the viscose to the spinneret, to produce the filaments of irregular denier, are shown in U. S. Patents Nos. 2,142,597 and 2,065,124.

By the continuous two-bath process of the invention the fibers are produced at substantially no increase in cost as compared to the cost of manufacturing regenerated cellulose fibers by conventional procedures utilizing a single coagulating and regenerating bath. Sulfuric acid is consumed for neutralizing substantially all of the sodium hydroxide introduced into the coagulating bath; the phosphate radicals are circulated in the system and serve as a vehicle for the hydrogen ions derived from the sulfuric acid, the only loss being a small one incidental to removal of the phosphate radicals from the regenerating bath with the yarn, which may be recovered if desired; there is substantially no mechanical loss of sulfuric acid by removal in stream 4, which contributes materially to the economical operation of the process; ready control of all variables is possible; and the circulating system is entirely self-regulating.

In the embodiments of the invention which have been described in detail, sodium sulfate is used as the dehydrating agent in the coagulating bath throughout the spinning, and for reasons of economy and simplicity, this is preferred. However, other dehydrating agents which are useful in the coagulation of viscose may be present in the coagulating bath at the start, and preferably those dehydrating agents which are stable under the pH conditions existing in the coagulating bath and in the regenerating bath. Examples of other suitable dehydrating agents are sodium chloride and magnesium sulfate. During spinning, such agents are gradually replaced by sodium sulfate.

Since some variations may be made in the process as set forth in specific detail in the examples, it is to be understood that the invention is not to be limited except as defined in the appended claims.

We claim:

1. A method for the production of shaped articles of regenerated cellulose from viscose which comprises extruding viscose into an aqueous coagulating bath having a pH of 1.5 to 10 and containing a dehydrating agent for viscose and inorganic phosphate radicals at least some of which are in the form of a sodium salt, withdrawing the cellulose xanthate article thus formed from the bath, passing the cellulose xanthate article carrying adhering coagulating solution to and through an aqueous cellulose-regenerating bath comprising an equilibrium mixture of the dehydrating agent and phosphoric acid, and sulfuric acid to convert to phosphoric acid at least part of the phosphate salts in the article, stretching the article at some time between coagulation and complete regeneration of the cellulose, continu-

## 11

ously passing excess regenerating bath built up during the spinning to the coagulating bath in a controlled amount so correlated with the amount of coagulating solution carried into the regenerating bath by the cellulose xanthate article that the pH balance in the coagulating bath is not upset, and removing from the coagulating bath by evaporation and crystallization water and sodium sulfate built up in said bath during the extrusion of the viscose, the composition and pH of the coagulating bath being maintained substantially constant from the beginning to the end of the extrusion.

2. A method for the production of shaped articles of regenerated cellulose from viscose which comprises extruding viscose into an aqueous coagulating bath having a pH of 1.5 to 10 and containing sodium sulfate and inorganic phosphate radicals at least some of which are in the form of a sodium salt, withdrawing the cellulose xanthate article thus formed from the bath, passing the cellulose xanthate article carrying adhering coagulating solution to and through an aqueous cellulose-regenerating bath comprising an equilibrium mixture of sodium sulfate and phosphoric acid, and sulfuric acid to convert to phosphoric acid at least part of the phosphate salts in the article, stretching the article at some time between coagulation and complete regeneration of the cellulose, continuously passing excess regenerating bath built up during the spinning to the coagulating bath in a controlled amount so correlated with the amount of coagulating solution carried into the regenerating bath by the cellulose xanthate that the pH balance in the coagulating bath is not upset, and removing from the coagulating bath by evaporation and crystallization water and sodium sulfate built up in said bath during the extrusion of the viscose, the composition and pH of the coagulating bath being maintained substantially constant from the beginning to the end of the extrusion.

3. A method for the production of shaped articles of regenerated cellulose from viscose which comprises extruding viscose into an aqueous coagulating bath having a pH of 1.5 to 10 and containing phosphate radicals at least some of which are in the form of a sodium salt, withdrawing the cellulose xanthate article thus formed from the bath, passing the cellulose xanthate article comprising adhering coagulating solution to and through an aqueous cellulose-regenerating bath comprising an equilibrium mixture of sodium sulfate and phosphoric acid, and sulfuric acid to convert to phosphoric acid at least part of the phosphate salts in the article, stretching the article at some time between coagulation and complete regeneration of the cellulose, continuously passing excess regenerating bath built up during the spinning to the coagulating bath in a controlled amount so correlated with the amount of coagulating solution carried by the article into the regenerating bath that the pH balance in the coagulating bath is not upset, adding to the coagulating bath predetermined amounts of sulfuric and phosphoric acids from a source other than the regenerating bath, and removing from the coagulating bath by evaporation and crystallization water and sodium sulfate built up in said bath during extrusion of the viscose, the composition and pH of the coagulating bath being maintained constant from the beginning to the end of the extrusion.

4. A method for the production of regenerated cellulose fibers from viscose which comprises ex-

## 12

truding viscose through a spinneret into an aqueous coagulating bath having a pH from 1.5 to 10 and containing sodium sulfate and inorganic phosphate radicals at least some of which are in the form of a sodium salt, withdrawing the cellulose xanthate fibers thus formed from the bath, passing the cellulose xanthate fibers carrying adhering coagulating solution to and through an aqueous cellulose-regenerating bath comprising an equilibrium mixture of sodium sulfate and phosphoric acid, and sulfuric acid to convert to phosphoric acid at least part of the phosphate salts in the fibers, stretching the fibers at some time between coagulation and complete regeneration of the cellulose, continuously passing excess regenerating bath built up during the spinning to the coagulating bath in a controlled amount so correlated with the amount of coagulating solution carried by the fibers into the regenerating bath that the pH balance in the coagulating bath is not upset, supplementing the sulfuric acid and phosphoric acid introduced into the coagulating bath from the regenerating bath with predetermined amounts of sulfuric and phosphoric acids from a source other than the regenerating bath, removing from the coagulating bath by evaporation and crystallization water and sodium sulfate built up in said bath during extrusion of the viscose, the composition and pH of the coagulating bath being maintained substantially constant from the beginning to the end of the extrusion, withdrawing the fibers from the regenerating bath, after-treating the fibers, and drying the fibers.

5. A method as in claim 1, in which the cellulose xanthate articles are stretched between the coagulating bath and the aqueous cellulose-regenerating bath and relaxed during passage thereof through the regenerating bath.

6. A method as in claim 1 in which the cellulose xanthate articles are stretched as they are passed through the aqueous cellulose-regenerating bath.

7. A method as in claim 2, in which the cellulose xanthate article carries adhering coagulating solution in an amount of not more than 8 parts by weight of solution per part of cellulose into the regenerating bath, and all of the excess regenerating bath produced during the spinning operation is passed continuously to the coagulating bath.

8. A method as in claim 2, in which the viscose has a ball fall viscosity of from 65 to 120 seconds.

9. A method as in claim 2, wherein the coagulating bath contains, by weight, from 5 to 20% phosphate radicals, from 5 to 22% sodium sulfate, and has a pH from 1.5 to 10.

10. A method as in claim 3, in which the cellulose xanthate articles are stretched between the coagulating bath and the aqueous cellulose-regenerating bath, and relaxed during passage thereof through the regenerating bath.

11. A method as in claim 3, in which the cellulose xanthate articles are stretched as they are passed through the aqueous cellulose-regenerating bath.

12. A method as in claim 3, in which the cellulose xanthate article leaving the coagulating bath is stripped of adhering coagulating solution to such an extent that not more than 8 parts by weight of solution from the coagulating bath per part of cellulose are carried with the article into the regenerating bath, and all of the excess regenerating bath produced during the spinning

75

operation is passed continuously to the coagulating bath.

13. A method as in claim 3, wherein the viscose has a ball fall viscosity of from 65 to 120 seconds.

14. A method as in claim 3, wherein the coagulating bath contains, by weight, from 5 to 20% phosphate radicals, from 5 to 22% sodium sulfate, and has a pH from 1.5 to 10.

15. A method as in claim 4, wherein the fibers are stretched between the coagulating bath and 10 the regenerating bath, and relaxed during passage thereof through the regenerating bath.

16. A method as in claim 4, wherein the fibers are stretched as they enter the regenerating bath.

17. A method as in claim 4, wherein the fibers 15 are stretched as they are passed through the regenerating bath.

18. A method as in claim 4, wherein the fibers are stretched at least 40%.

19. A method as in claim 4, wherein the fibers 20 are given a stretch of from 100% to 200%.

20. A method as in claim 4, wherein the viscose is extruded into the coagulating bath at an extrusion rate of at least four times the velocity of draw-off, stretched between the coagulating bath and the aqueous cellulose-regenerating bath, relaxed during passage thereof through the regenerating bath, withdrawn from the regenerating bath, after-treated, and dried in relaxed condition.

GEORGE A. RICHTER, JR.  
RICHARD H. BRAUNLICH.

#### REFERENCES CITED

The following references are of record in the file of this patent:

#### UNITED STATES PATENTS

| Number    | Name         | Date          |
|-----------|--------------|---------------|
| 2,236,648 | Nagel et al. | Apr. 1, 1941  |
| 2,512,968 | Ray          | June 27, 1950 |